

July 29, 1924.

1,502,763

L. W. BUGBEE

PENCIL AND PROCESS OF MAKING THE SAME

Filed Jan. 18, 1924

FIG. 1



FIG. 2



FIG. 3



FIG. 4



FIG. 5



INVENTOR.  
LUCIAN W. BUGBEE.

BY

*Lucian W. Bugbee*

ATTORNEYS.

## UNITED STATES PATENT OFFICE.

LUCIAN W. BUGBEE, OF INDIANAPOLIS, INDIANA.

## PENCIL AND PROCESS OF MAKING THE SAME.

Application filed January 18, 1924. Serial No. 687,032.

*To all whom it may concern:*

Be it known that I, LUCIAN W. BUGBEE, a citizen of the United States, and a resident of Indianapolis, county of Marion, 5 and State of Indiana, have invented a certain new and useful Pencil and Process of Making the Same; and I do hereby declare that the following is a full, clear, and exact description thereof, reference being had to the accompanying drawings, in which like numerals refer to like parts.

The object of this invention is the provision of a pencil in which the pores of the lead are filled with coloring matter or ink 15 which will afford any desired coloring of writing and will make the same permanent. One feature of the invention consists in the process of making such lead pencil by mixing clay and wood dust or other oxidizable 20 material in forming the lead and then heating the lead in such manner as to consume or oxidize the wood dust and leave the lead consisting of clay honeycombed with pores, and then filling the lead by saturating it in 25 a melted solution of wax and pigment of the desired color until the pores are filled.

I am aware that colored pencils have heretofore been made, but not with the hard vitrified honeycombed clay structure as 30 herein set forth. With my invention I have a lead as hard as the ordinary lead pencil instead of the soft easily breakable colored leads in common use. Also the hardness can be controlled by the proper proportions of 35 clay and by the firing temperature.

The full nature of the invention will be understood from the accompanying drawings and the following description and claims:

40 In the drawings, Figure 1 is a plan view of the lead pencil with the end broken away. Fig. 2 is a similar view of the lead with the end broken away. Fig. 3 is a plan view of a part of Fig. 2, very greatly enlarged and 45 showing the mixture of clay and wood dust. Fig. 4 is the same showing it after the wood dust has been oxidized or consumed and leaving the clay porous. Fig. 5 is the same after the porous clay has been filled with a 50 color.

In making the pencil herein set forth the first step in the process is to mix clay 8 and wood dust 9 or the like into a plastic composition and for that purpose the proportions 55 may be one of clay and two of wood dust,

but the invention is not limited to any exact proportions.

The second step in the process is to extrude the leads 10 from this plastic mass. The third step of the process consists in 60 heating the leads in such way as to consume or oxidize the wood dust or other carbonaceous material and harden the clay and leave the latter honeycombed with pores. This is done by placing the leads in an open 65 crucible and heating it sufficient to oxidize and burn out all the carbon and leave only the honeycombed hard clay structure. This leaves the lead as shown in Fig. 4.

The fourth step in the process consists in 70 saturating the honeycombed clay lead in a colored solution of wax-like material and a pigment of desired color, which were previously intermixed, until the pores in the clay are filled with the pigment and wax 75 and the lead coated with the latter.

By this invention a lead is produced that is as hard as the ordinary lead pencil instead of the soft easily breakable colored 80 leads in common use and the hardness can be increased by increasing the proportion of clay and the firing.

The filling may include a solution of silver nitrate, copper chloride or other suitable chemical to act on the structure of the 85 paper and that will make erasure or alteration in signature or writing impossible. The color pigment may be such that it is capable of producing the desired color chemically or by the action of the light. 90

The invention claimed is:

1. The process of making a pencil, which process includes forming a lead of clay and carbonaceous material intermixed, second in heating said lead so as to oxidize the carbonaceous material and leave a lead formed of hard honeycombed clay, and afterwards filling said lead with colored pigment. 95

2. The process of making a pencil, which process includes forming a lead of clay and carbonaceous material intermixed, second in heating said lead so as to oxidize the carbonaceous material and leave a lead formed of hard honeycombed clay, forming a solution of colored pigment and wax-like material, and saturating said honeycombed clay lead therein so as to fill and coat the same. 100

3. The process of making a pencil, which process includes forming a lead of clay and wood dust intermixed in substantially the 110

proportion of one part of clay and two parts of wood dust intermixed in plastic form, extruding leads from said plastic mass, baking said leads until the wood is 5 oxidized and removed, forming a solution of colored pigment and wax-like material, and saturating the leads therein to fill and coat the same.

4. The process of making a pencil, which 10 process includes forming a lead of clay and carbonaceous material intermixed, second in baking said lead so as to oxidize the carbonaceous material and leave the lead formed of hard honeycombed clay, forming

a filler including a chemical that will act 15 on the structure of the paper, and saturating said honeycombed clay lead therein so as to fill the same.

5. A pencil having a lead formed of honeycombed clay, and a filling of colored 20 pigment and wax-like material.

6. A pencil having a lead formed of honeycombed clay, and a filling which will act as a chemical on the structure of the paper in order to make an erasure thereof impossible. 25

In witness whereof I have hereunto affixed my signature.

LUCIAN W. BUGBEE.